

Sept. 15, 1931.

H. LANGWELL

1,823,691

GRINDING OF CELLULOSIC MATERIALS

Filed July 9, 1928



Inventor:  
Herbert Langwell  
By Bonifant Hamilton, Atty

## UNITED STATES PATENT OFFICE

HERBERT LANGWELL, OF EPSOM, ENGLAND, ASSIGNOR TO COMMERCIAL SOLVENTS CORPORATION, OF TERRE HAUTE, INDIANA, A CORPORATION OF MARYLAND

## GRINDING OF CELLULOUS MATERIALS

Application filed July 9, 1928. Serial No. 291,212.

The present invention relates to a method of grinding or comminuting various materials, and it is especially adapted to the grinding of cellulosic or plant material which possesses a relatively soft portion and a relatively hard and tough portion which normally has given rise to much difficulty in the comminution of such material, especially in cases where it is desired to produce a fairly fine and homogeneous ground product.

The invention is particularly adapted to the grinding of corncobs preparatory to the fermentation thereof, or for other purposes, but it will be understood that the process may be equally applied to any cellulosic material of the nature above outlined; and, although the grinding of corncobs is herein specifically illustrated, nevertheless, this adaptation is illustrative only.

In recent years industrial demands for fermentation products of cellulose have so greatly increased that it has been found highly expedient, in view of the decreasing supply of the raw materials commonly employed for these purposes, to seek a cheap and relatively constant supply of cellulose, and in view of the fact that corn is one of the principal staple crops of the United States, much investigation attended with marked success has been made of the utilization of the cellulose of corncobs as a substitute for wood, as a source of valuable products in high demand by the industries.

It may here be pointed out that the structure of a corncob consists of a soft outer layer surrounding a hard, tough core, and that the efficient fermentation of the cobs requires a relatively fine and homogeneous meal, which meal is produced by the grinding of the cobs. This grinding operation has heretofore normally been attended with marked difficulties: The hard, tough core prevents, normally, grinding the cobs in rolls, as the rolls become choked and blocked by the tough core; the grinding must therefore be done by attrition, and the hard, tough core causes a very high degree of wear upon the mills, and even then there is frequently not an even grinding of the core material, as its tendency is to flake instead of grinding to a meal.

The present invention seeks to overcome these difficulties of dry grinding by overcoming the flaking tendency of the core, and rendering the entire cob thoroughly brittle, thereby permitting the use of rolls in grinding, and very materially reducing the wear in attrition mills.

The invention is predicated upon the fact that dry cobs are brittle, the brittleness increasing with reduction of the moisture content of the cobs. It has been found that if the cobs are substantially heated, but insufficiently to char them, and then ground while they are in a substantially heated condition, the above objects are attained, as the moisture content is reduced to a low minimum by the heating, and reabsorption of moisture is prevented. The cobs therefore have a maximum degree of brittleness and can be readily reduced to a homogeneous meal, with a relatively low power consumption.

In carrying out the drying, any type of drier, which may be convenient, can be employed. The accompanying drawing illustrates one form which has been found to be efficient, the single figure representing a diagrammatic sectional view of a vertical shaft type of kiln.

Referring in detail to the drawing, the kiln is generally indicated at 10, and is provided with ports, 11, adapted to admit heated gases for the carrying out of the drying. For heating these gases, there is provided a stove, 12, conveniently heated by burning coke, indicated at 13. It will be understood that any convenient type of heater, and any convenient kind of fuel may be employed in the place of the specific illustrated type of heater. In the illustrated installation, air may be admitted to the stove or heater, 12, through the line, 14, the line conveniently branching, as indicated at 15 and 16, so as to admit air above and below the coke bed, 13, as desired, dampers, 17 and 18, being placed in the branches, 15 and 16, respectively, to direct the flow of air through the stove as desired.

It may be here pointed out that the kiln, 10, is a vertical open shaft type of kiln, the charge being indicated by the numeral 19, this

charge being the cellulosic material or corn-cobs which are to be dried.

In operation, the cellulosic material or cobs are first air dried, and then periodically charged into the top of the open shaft and removed from the base in equivalent amounts so as to keep a constant depth of charge in the shaft. A coke fire in the stove, 12, supplies hot flue gases, which, when mixed with an excess of cold air introduced through the branch, 15, to give a mixture of gases at, say 110° C., are blown through the charge in the shaft in a direction opposite to the movement of the charge at such a rate that moisture is not deposited on the cold newly charged material at the top of the shaft. Precautions should be taken to prevent sparks from the coke fire reaching the charge and firing it. The charge is introduced into the mill for grinding while hot, absorption of moisture being thereby prevented.

As a specific illustration of the process as applied to the grinding of corncobs, the following example is given:

25 A batch of steam-dried cobs which had been crushed to a moderate degree of fineness (4 to 2 mesh) were heated until they began to scorch. Half of the lot was put into cans with tight covers and allowed to cool. The other half was ground hot in a fine pulverizer, the temperature of the feed to the pulverizer varying from about 160° to 180°. The results of the grind were as follows:

| 35 | Run number.....             | 1.....       | 2.....                       |
|----|-----------------------------|--------------|------------------------------|
|    | Temperature of cobs.....    |              | Mill temperature.....        |
|    | Rate of grinding.....       | 203 lbs./hr. | 160°-180° C.<br>240 lbs./hr. |
|    | Screen analysis of product: |              |                              |
| 40 | On 8 mesh.....              | 22½          | 23½                          |
|    | On 14 mesh.....             | 25           | 25                           |
|    | On 20 mesh.....             | 8            | 9                            |
|    | On 28 mesh.....             | 8            | 11½                          |
|    | On 48 mesh.....             | 15½          | 15½                          |
|    | On 100 mesh.....            | 10           | 9                            |
|    | Through 100 mesh.....       | 10           | 6½                           |

These results indicate an increased grinding capacity of approximately 20% when the cobs are hot.

The hot grinding acts upon the cobs when they have their maximum degree of fragility, and increases the advantages of dry grinding, as there is no possibility of reabsorption of moisture and the moisture content of the hot cobs is the absolute minimum which is possible. Before dry grinding was applied to corncobs, wet digestion processes were tried but were abandoned for the dry grinding process on account of the difficulty of wet grinding and the trouble which the pulp sometimes caused in the fermenter. Taking into consideration the cost of digestion, the trouble in handling and grinding wet material, and the complication due to furfural and slimy washes, wet grinding has been discontinued in favor of dry grinding. The dry grinding avoided these difficulties, although in the latter there is somewhat of an

increase in the power consumption required, owing to the structure of the cobs; and also, it was extremely difficult to get a uniformly ground meal. These disadvantages are largely overcome through the application of hot grinding, as herein described.

With respect to dry grinding of cobs, the following procedure and data are illustrative of this process:

Five batches of cobs of apparently different moisture content were selected. These were each put through a preliminary crusher, and then a weighed amount of each batch was run through a fine pulverizer. Each batch was carefully weighed and scrubbed before and after going through the pulverizer. The time of grinding was observed. Moisture was determined on the samples going to the pulverizer and screen analyses were made on the pulverizer product. The cobs are nearly dried in passing through the pulverizer.

| Sample No.....                             | 1.....      | 2..... | 3..... | 4a.....   | 4b.....   | 90  |
|--------------------------------------------|-------------|--------|--------|-----------|-----------|-----|
| Description.....                           | Dry cobs.   | Damp.  | Wet.   | Very wet. | Very wet. |     |
| Weight before grinding.....                | 50 lbs..... | 50     | 50     | 50        | 50        |     |
| Weight after grinding.....                 | 48 do.....  | 46     | 43     | 38        | 38        |     |
| Time of grinding.....                      | 28 min..... | 43     | 60     | 105       | 99        | 95  |
| Screen analyses:                           |             |        |        |           |           |     |
| On 8 mesh.....                             | 26½         | 35     | 33     | 20        | 19        |     |
| On 14 mesh.....                            | 26½         | 31     | 28     | 38½       | 40        |     |
| On 20 mesh.....                            | 12½         | 10     | 9½     | 10        | 12½       |     |
| On 28 mesh.....                            | 11½         | 7      | 8½     | 7         | 9½        |     |
| On 48 mesh.....                            | 13½         | 9      | 9½     | 10        | 9½        |     |
| Through 100 mesh.....                      | 6           | 3      | 6      | 6         | 3         |     |
| Residue.....                               | 5           | 4      | 5      | 8         | 7         | 100 |
| Per cent H <sub>2</sub> O (wet basis)..... | 5.3%        | 11     | 14.6   | 26.5      | 27.4      |     |

#### Calculations

| Sample No.....                     | 1.....                             | 2.....                          | 3.....                           | 4a.....                               | 4b.....                               | 105 |
|------------------------------------|------------------------------------|---------------------------------|----------------------------------|---------------------------------------|---------------------------------------|-----|
| Description.....                   | Dry cobs.<br>(5% H <sub>2</sub> O) | Damp.<br>(11% H <sub>2</sub> O) | Wet.<br>(14.6% H <sub>2</sub> O) | Very wet.<br>(26.5% H <sub>2</sub> O) | Very wet.<br>(27.4% H <sub>2</sub> O) |     |
| Mill temperature.....              | warm.                              | warm.                           | warm.                            | cold.                                 | warm.                                 | 110 |
| Grinding rate wet cobs.....        | 107 lbs./hr.                       | 70                              | 50                               | 28½                                   | 30½                                   |     |
| Grinding rate dry cobs.....        | 101 lbs./hr.                       | 62                              | 43                               | 21                                    | 22                                    |     |
| Lbs./hr. through 8 mesh.....       | 74½                                | 40                              | 29                               | 17                                    | 18                                    |     |
| Lbs. per hrs. through 20 mesh..... | 35                                 | 17                              | 12½                              | 6½                                    | 6½                                    | 115 |

From the above data, it will be seen that the grinding rate very rapidly increases with the reduction of the moisture content of the cobs. For wet cobs having a moisture content of 20%, the grinding rate will be about 35 lbs. per hour; reduction to 10% moisture increases the grinding rate to 75 lbs. per hour; and reduction to 5% gives a grinding rate of 107 lbs. per hour, or 101 lbs. of actual cob (95% of 107 lbs., since there is 5% moisture present).

This shows, therefore, that the rate of grinding of such materials as corncobs is

greatly increased through reduction of the moisture content; and the grinding of the cobs while hot gives the maximum grinding efficiency. This is of importance in any connection where a uniform meal is desired, and the time factor is of importance.

It will be understood that the above specific examples are illustrative only of the invention, and that it is desired to comprehend within the scope of this invention such modifications and changes as may be necessary to adapt it to varying conditions and uses.

What is claimed is:

1. A process of grinding cellulosic material which comprises heating the material sufficiently high to expel the moisture therefrom but avoiding substantial charring, and then immediately grinding the said material before substantial cooling thereof.

2. A process of grinding corncobs which comprises heating the cobs to a temperature ranging from approximately 110° C. to approximately 180° C. until substantially all moisture is expelled, and then immediately grinding the cobs before substantial cooling thereof.

3. A process of grinding corncobs which comprises heating the cobs sufficiently high to expel the moisture therefrom but avoiding substantial charring, and then immediately grinding the said material before substantial cooling thereof.

4. A process of grinding cellulosic material which comprises heating the material to a temperature ranging from approximately 110° C. to approximately 180° C., until substantially all moisture is expelled, and then immediately grinding the material before substantial cooling thereof.

5. A process of grinding cellulosic material which comprises heating the material sufficiently high to reduce the moisture content of said material to below approximately 5% but avoiding substantial charring, and then immediately grinding the said material before substantial cooling thereof.

6. A process of grinding corncobs which comprises heating said cobs sufficiently high to reduce the moisture content of the cobs to below approximately 5%, and then immediately grinding the cobs before substantial cooling thereof.

7. A process of grinding cellulosic material which comprises heating said material to a temperature ranging from approximately 110° C. to approximately 150° C. until the moisture content is reduced to below approximately 5%, and then immediately grinding the said material before substantial cooling thereof.

8. A process of grinding corncobs which comprises heating the cobs to a temperature range from approximately 110° C. to approx-

imately 180° C. until the moisture content is reduced to below approximately 5%, and then immediately grinding the cobs before substantial cooling thereof.

In testimony whereof I affix my signature.

HERBERT LANGWELL.